

Patented Jan. 16, 1934

1,943,377

# UNITED STATES PATENT OFFICE

1,943,377

## TREATMENT OF CELLULOSE ESTERS

George Holland Ellis, Spondon, near Derby, England, assignor to Celanese Corporation of America, a corporation of America

No Drawing. Application December 21, 1928, Serial No. 327,759, and in Great Britain January 30, 1928

7 Claims. (Cl. 95—6)

This invention relates to the production of effects (photographic or otherwise) on fabrics, films or other materials made of or containing cellulose acetate or other cellulose esters, for example cellulose formate, propionate or butyrate.

I have found that the extraordinary ease with which amines may be incorporated in cellulose ester materials enables the known light-sensitivity of diazo compounds to be utilized to obtain upon such materials successful photographic or pattern effects which are exceedingly fast to washing and which, by a suitable choice of components may be very fast to other agencies. Moreover the "prints" or impressions are not merely superficial.

According to the present invention therefore materials comprising cellulose acetate or other cellulose esters and containing diazotizable amino compounds are diazotized, the materials then exposed to the action of light of locally varying intensity and the pattern or effect fixed by development with one or more components capable of converting the diazo body into an azo compound.

The diazotizable amino compounds, which may be simple amines or aminoazo compounds and may be coloured or not, may be incorporated in the fabric, film or other material by any suitable means, but are preferably applied by immersing the material in an aqueous solution or dispersion. Aqueous solutions of salts, e. g. the hydro-chlorides, may be employed or aqueous solutions of the free bases where these are sufficiently soluble. If insufficiently soluble the amines may still be applied as free bases in aqueous dispersions obtained by any suitable means, for example by grinding (e. g. in the so-called colloid mills) in presence or absence of dispersors or protective colloids, by dissolving in a solvent and mixing the solution with water containing or not containing dispersors or protective colloids, or by pretreating the bases with suitable dispersors for example by the methods described in prior U. S. patents to Ellis Nos. 1,618,413 and 1,618,414 of

February 22, 1927, No. 1,694,413 of December 11, 1928, No. 1,716,721 of June 11, 1929, and to Ellis and Goldthorpe No. 1,690,481 of June 6, 1928, and Ellis U. S. application Serial No. 134,138 filed September 7, 1926, and Ellis and Goldthorpe U. S. application Serial No. 152,517 filed December 3, 1926.

Alternatively suitable amino bases may be applied from solution in organic solvents, for instance trichlorethylene, the solvent or solvent mixture being so chosen that it has no deleterious effect upon the cellulose ester. Again the amino bases may be incorporated in the cellulose ester solution employed to manufacture the films, filaments or other products.

The cellulose-ester-organic-base complex is

subjected to diazotization to convert the amine into the diazo form, preferably under conditions so that the light is so subdued, coloured or excluded that the diazo compound is unaffected. The material is preferably then dried under these restricted light conditions and under comparatively cool or cold conditions. If the diazo compound is itself sufficiently stable or if stabilizers be employed, the dried material containing the "active" diazo compound may be stored for future exposure and development. The invention includes these dry materials containing the stable diazo compound.

On the fabric, film or other material thus prepared a light impression may now be obtained by any suitable means, for example by direct photography of the object in the usual way by employment of any form of camera, or by employment of any form of "positive" or "negative" or stencil or other device whereby the reflected or transmitted light incident on the material is locally varied in intensity so as to yield a design or picture as required. Exposure conditions will of course vary according to the diazo compound (or mixture) employed.

After a suitable exposure the material is subjected to the development process, the developer being applied in dispersed or other form.

The following are examples of suitable amino compounds and developers for use according to the present invention, but it is to be understood that the listing of these examples implies no limitation of the invention thereto:—

| A. | Amino compounds                                                                                                                      | 95  |
|----|--------------------------------------------------------------------------------------------------------------------------------------|-----|
|    | p-Nitraniline                                                                                                                        |     |
|    | p-Nitro-o-anisidine                                                                                                                  |     |
|    | m-Nitro-p-toluidine                                                                                                                  |     |
|    | m-Nitro-o-anisidine                                                                                                                  |     |
|    | p-Chloraniline                                                                                                                       | 100 |
|    | $\alpha$ -Naphthylamine                                                                                                              |     |
|    | Benzidine                                                                                                                            |     |
|    | Dianisidine                                                                                                                          |     |
|    | p-Aminobenzene-azo- $\alpha$ -naphthylamine                                                                                          |     |
| B. | Developers                                                                                                                           | 105 |
|    | $\alpha$ -Naphthylamine                                                                                                              |     |
|    | Dimethylaniline                                                                                                                      |     |
|    | m-Phenylenediamine                                                                                                                   |     |
|    | $\alpha$ -Naphthol                                                                                                                   | 110 |
|    | $\beta$ -Naphthol                                                                                                                    |     |
|    | Phenol                                                                                                                               |     |
|    | $\beta$ -Oxynaphthoic acid                                                                                                           |     |
|    | p-Xylylidine                                                                                                                         |     |
|    | $\beta$ -Naphthylamine                                                                                                               | 115 |
|    | Aminonaphthols                                                                                                                       |     |
|    | Acetoacetic ester.                                                                                                                   |     |
|    | Mixtures of organic bases and/or mixtures of developers may be employed and by employing combinations of diazo compounds which react | 120 |

differently to light and yield different shades with the same or with mixed developers, wide varieties of effects are obtainable.

If desired, the materials may previously be dyed with, or may otherwise have incorporated therein, colouring matters which resist the diazotization process and the exposure to light, or alternatively colouring matters may be applied to the materials after the process of the present invention. By this means effects or designs are obtainable on a contrasting or shading background.

The following examples are intended to illustrate the invention, but not to limit it in any way:—

15

*Example 1*

A satin fabric woven from cellulose acetate yarns is "dyed" with 1% of its weight of dianisidine which has been previously dispersed by heating with five times its weight of sodium sulphorcinolate before adding to the dyebath. The "dyeing" is continued for 1½ hours at 80° C., after which the fabric is rinsed well in warm water and diazotized in a bath containing 2% sodium nitrite and 7% hydrochloric acid 32° Tw., calculated on the weight of fabric. After diazotizing for half an hour at room temperature the material is rinsed very well in cold water and dried. The drying, which is preferably effected on some stretching device to avoid creases in the fabric, is carried out in subdued light while maintaining the fabric fairly cool.

A piece of the dry diazotized fabric is placed in a photographic printing frame behind a transparent positive image and exposed for the necessary time to sunlight or the carbon arc, after which it is "developed" in a bath containing 1.5% of methaphenylene diamine, calculated on the weight of fabric. The developing bath is raised from cold to 60° C. in ½ hour and maintained at 60° C. for ½ hour. The material is finally rinsed, soaped lightly and dried. A bright scarlet photograph is obtained on a very pale cream ground.

45

*Example 2*

A woven fabric composed of cellulose acetate yarns is "dyed" in a dyebath of volume ratio 50 to 1 with 2% of its weight of 2:amino-5-nitro-methoxybenzene, previously solubilized by heating with five times its weight of sodium sulphorcinolate. After dyeing for 1½ hours at 80° C. the fabric is rinsed in warm water and diazotized and dried as in Example 1. It is exposed under a stencil or transparent photographic "positive" to sunlight or the arc light for the necessary time after which it is developed in 3% of 2,3-oxynaphthoic acid, calculated on the weight of fabric, the developer having been dispersed in the dye-bath by dissolving in the minimum of caustic soda, pouring into the bath containing 5% glue on the weight of goods, and carefully neutralizing with formic acid. The developing bath is raised to 60° C. in ½ hour and maintained at 60° C. ½ hour, after which the "print" is rinsed well, soaped lightly and dried. A bright bluish red design or photograph on a buff ground is thus obtained.

70

*Example 3*

A woven fabric composed of cellulose acetate yarns is "dyed" as in Example 1 with 1% of its weight of dianisidine and diazotized in the manner given: The dried diazotized fabric is exposed under a stencil or a transparent positive photographic image to sunlight or the electric arc for the necessary time and developed in a mixture of dimethylaniline and 2,3-oxynaphthoic acid. 1.5% 2,3-oxynaphthoic acid on the weight of fabric is dispersed as in Example 2, and 1% dimethylaniline is dispersed by heating with sodium sulphorcinolate before adding to the developing bath. The print is developed in the mixed developers, raising to 60° C. in ½ hour and maintaining at 60° C. ½ hour. It is finally rinsed, soaped lightly and dried. A purple-brown design or photograph is obtained on a pale buff ground.

What I claim and desire to secure by Letters Patent is:—

1. Process for the production of pattern effects, comprising diazotizing a material comprising a cellulose ester containing a diazotizable amine, exposing to the action of light of locally varying intensity and fixing the pattern by development.

2. Process for the production of pattern effects, comprising diazotizing a material comprising a cellulose ester containing a diazotizable amine, drying, exposing to the action of light of locally varying intensity and fixing the pattern by development.

3. Process for the production of pattern effects, comprising diazotizing a material comprising cellulose acetate containing a diazotizable amine, exposing to the action of light of locally varying intensity and fixing the pattern by development.

4. Process for the production of pattern effects, comprising diazotizing a material comprising cellulose acetate containing a diazotizable amine, drying, exposing to the action of light of locally varying intensity and fixing the pattern by development.

5. Process for the production of photographic effects, comprising diazotizing a material comprising cellulose acetate containing a diazotizable amine, exposing to the action of light passing through a photographic positive and fixing the photographic image by development.

6. Process for the production of pattern effects, comprising diazotizing a material comprising a cellulose ester containing a substantially colorless diazotizable amine, exposing to the action of light of locally varying intensity and fixing the pattern by development.

7. Process for the production of pattern effects, comprising diazotizing a material comprising cellulose acetate containing a substantially colorless diazotizable amine, drying, exposing to the action of light of locally varying intensity and fixing the pattern by development.

GEORGE HOLLAND ELLIS.

140

145

**CERTIFICATE OF CORRECTION.**

**Patent No. 1,943,377.**

**January 16, 1934.**

**GEORGE HOLLAND ELLIS.**

It is hereby certified that the State of Incorporation of the assignee in the above numbered patent was erroneously described and specified as "America" whereas said State of Incorporation should have been described and specified as Delaware, as shown by the records of assignments in this office; page 2, line 38, for "methaphenylene" read metaphenylene; and that the said Letters Patent should be read with these corrections therein that the same may conform to the record of the case in the Patent Office.

Signed and sealed this 6th day of March, A. D. 1934.

**F. M. Hopkins**

**(Seal)**

**Acting Commissioner of Patents.**